

1

3,148,055

## ZIRCONIUM ALLOYS

Stanley Kass, Pittsburgh, Wilbert W. Kirk, Wilkinsburg, and Donald W. Bright, Pittsburgh, Pa., assignors to Westinghouse Electric Corporation, East Pittsburgh, Pa., a corporation of Pennsylvania  
No Drawing. Filed Apr. 14, 1960, Ser. No. 22,133  
3 Claims. (Cl. 75—177)

This invention is directed to novel zirconium alloys having high resistance to corrosion and good mechanical strength.

In U.S. Patent No. 2,772,964, issued December 4, 1956, and assigned to the assignee of the present invention, there are disclosed alloys of zirconium that are characterized by highly desirable properties for many applications. The alloys of this U.S. patent have excellent properties at room temperature and at elevated temperatures and have therefore found wide application in industry, particularly in an environment of hot water or steam.

Zirconium and its alloys are, almost without exception, subject to corrosion to a greater or lesser degree in the presence of hot water or steam. One of the products of the corrosion reaction is hydrogen, and it has been found that this hydrogen is absorbed by the remaining zirconium alloy mass. The absorbed hydrogen adversely affects the mechanical strength of the members formed from the zirconium alloy. The decrease in mechanical strength accelerates the failure of members which may have suffered corrosion to a relatively insignificant degree.

It is accordingly an object of the present invention to provide zirconium-base alloys which possess good corrosion resistance, and in addition, have a decreased capacity for the absorption of hydrogen; the alloys including in predetermined proportions the elements tin, chromium, iron, oxygen and zirconium.

Another object of the invention is to provide a zirconium-base alloy consisting of from 0.1% to 2.5%, by weight tin, a total of from 0.1% to 2% by weight of at least one metal from the group consisting of iron, nickel, and chromium, from 0.16% to 0.25%, by weight, oxygen, the alloy exhibiting good corrosion resistance to high temperature water and steam, high strength, and good ductility. Some benefits are obtained if the oxygen content is slightly below 0.16%, though it must be at least 0.11%.

It is a further object of the invention to provide a zirconium-base alloy consisting of from 1.3% to 1.6%, by weight of tin, from 0.07% to 0.12%, by weight of chromium, from 0.12% to 0.40%, of iron, a maximum of 0.007% nickel, and small amounts of oxygen of from 0.16% to 0.25%, the alloy exhibiting good corrosion resistance to high temperature water and steam, high strength, and good ductility.

Other objects of the invention will, in part, be obvious and will, in part, appear hereinafter.

In accordance with the present invention, there are provided novel improved zirconium-base alloys characterized by high corrosion resistance to high temperature water and steam, good ductility, and low capacity for hydrogen absorption with resultant retention of high mechanical strength. These zirconium-base alloys consist essentially of from 0.1% to 2.5%, by weight of tin, a

2

total of from 0.1% to 2% by weight of at least one metal from the group consisting of iron, nickel, and chromium, at least 0.11%, but not exceeding 0.25%, by weight of oxygen, silicon not exceeding 0.012%, carbon not exceeding 0.05%, the balance being zirconium and less than 0.5%, by weight of incidental impurities such as nitrogen and carbon, as well as small amounts of non-detrimental elements.

An especially important alloy made in accordance with this invention is a family of alloys consisting essentially of from 1.3% to 1.6% by weight of tin, from 0.07% to 0.12% by weight of chromium, from 0.12% to 0.40% by weight of iron, at least 0.11%, but not exceeding 0.25% by weight of oxygen, nickel not exceeding 0.007%, carbon not exceeding 0.05%, the balance being zirconium and less than 0.5%, by weight of incidental impurities.

The alloys described above are particularly notable due to their low capacity for hydrogen absorption when exposed to high temperature water and steam. This characteristic results in the retention of high mechanical strength in such environments. Thus, the alloys may be employed in boilers and other apparatus wherein this particular combination of properties is advantageous.

The alloys of the present invention may be hot forged, hot rolled, hot extruded, or swaged from ingots thereof, even with substantial amounts of nitrogen of the order of 0.01% being present. Carbon may be present in amounts of up to 0.05%. The hot worked alloys may be readily cold worked to produce members of desired final size and shape.

The following examples are illustrative of the present invention. In these examples all parts and percentages given for a composition are by weight.

## EXAMPLE I

35 An alloy of the following composition was prepared:

|           | Percent      |
|-----------|--------------|
| Tin       | 1.3 to 1.6   |
| Chromium  | 0.07 to 0.12 |
| Nickel    | 0.04 to 0.08 |
| Iron      | 0.09 to 0.16 |
| Oxygen    | 0.125        |
| Zirconium | Balance      |

45 The nitrogen content did not exceed 50 parts per million and carbon was less than 0.05%. Corrosion test coupons of this alloy were prepared by shearing 0.030 inch thick cold-rolled strip into samples 1 inch x 1.5 inches and abrading the rough edges. The surfaces 50 were chemically etched to remove 0.002 inch per surface, thereby minimizing surface contamination.

The coupons were exposed to 680° F. water and 750° F. steam, atmospheres which are corrosive to the alloy, and the corrosion rate and hydrogen pick-up of the alloy 55 was measured. Similar coupons were made from a substantially identical alloy containing only 0.085% oxygen, and these coupons were also exposed to the same corrosive atmospheres. In the following Table I, the hydrogen pick-up of the two alloys is compared; the hydrogen pick-up values are presented as a ratio of the hydrogen absorbed by the alloys to the amount of hydrogen evolved in the corrosion reaction, in percent.

Table I

| Oxygen  | Days in 680° F. water |    |    |    |    |     |     |     |     |     | Days in 750° F. steam |    |    |    |    |    |     |     |
|---------|-----------------------|----|----|----|----|-----|-----|-----|-----|-----|-----------------------|----|----|----|----|----|-----|-----|
|         | 7                     | 14 | 28 | 56 | 84 | 112 | 140 | 168 | 196 | 224 | 7                     | 14 | 28 | 42 | 70 | 98 | 126 | 154 |
| 0.0850% | 33                    | 38 | 42 | 53 | 49 | 46  | 54  | 51  | 51  | 45  | 52                    | 42 | 42 | 49 | 47 | 52 | 57  | 54  |
| 0.1250% | 13                    | 23 | 18 | 22 | 13 | 14  | —   | —   | —   | —   | —                     | 31 | 32 | 32 | 42 | 33 | 29  | 22  |

A greatly decreased absorptive capacity for hydrogen is manifest in the higher oxygen alloys in Table I above. The mechanical strength of the high oxygen alloys greatly exceeded that of the low oxygen alloys.

It has been found in working with the alloys of the general type described above, that limiting the nickel content to a maximum value of 0.007% appreciably reduces the hydrogen pick-up. Modifications of this low nickel alloy involving variations in the iron content indicate that increasing iron contents to about 0.25% and higher increases the hydrogen pick-up. Again, the beneficial effect of oxygen in reducing or at least stabilizing the hydrogen pick-up can be demonstrated. The following Table II presents for a series of alloys having no significant nickel content, and in which the iron content was varied from a minimum of 0.120% to 0.336% while the oxygen content varied from a minimum of 0.090% to a maximum of 0.195%, the ratios (in percent) of the amount of hydrogen absorbed by the samples to that produced by the corrosion reaction.

capacity for hydrogen absorption during exposure to high temperature water or steam consisting of, from 0.1% to 2.5% by weight of tin, and a total of at least 0.1%, but not exceeding approximately 2% by weight of at least one metal from period 3 of the Periodic Table selected from the group consisting of iron, nickel, and chromium, at least 0.16%, but not exceeding 0.25%, by weight of oxygen, carbon not exceeding 0.05%, the balance being zirconium and less than 0.5% by weight of incidental impurities.

5 2. A zirconium-base alloy having a decreased ability to absorb hydrogen during exposure to high temperature water or steam consisting of, from 1.3% to 1.6% by weight of tin, from 0.07% to 0.12% by weight of chromium, from 0.04% to 0.08% by weight of nickel, from 0.09% to 0.16% by weight of iron, at least 0.16%, but not exceeding 0.25%, by weight of oxygen, carbon not exceeding 0.05%, the balance being zirconium and less than 0.5% by weight of incidental impurities.

10 3. A zirconium-base alloy having a decreased absorp-

Table II

|        | F <sub>2</sub> ,<br>percent | O <sub>2</sub> ,<br>percent | Days in 680° F. water |    |    |    |    |     |     |       |       |       |
|--------|-----------------------------|-----------------------------|-----------------------|----|----|----|----|-----|-----|-------|-------|-------|
|        |                             |                             | 7                     | 14 | 28 | 56 | 84 | 112 | 140 | 168   | 196   | 224   |
| 1----- | 0.1200                      | 0.090                       | 12                    | 16 | 13 | 15 | 16 | 16  | 16  | 16    | 14    | 13    |
| 2----- | 0.2400                      | 0.090                       | 20                    | 22 | 18 | 20 | 21 | 24  | 22  | 19    | 19    | 17    |
| 3----- | 0.2500                      | 0.170                       | 11                    | 17 | 15 | 14 | 21 | 19  | 19  | 17    | ----- | ----- |
| 4----- | 0.2800                      | 0.185                       | 14                    | 19 | 20 | 22 | 27 | 25  | 20  | 21    | ----- | ----- |
| 5----- | 0.3360                      | 0.195                       | 21                    | 16 | 18 | 25 | 27 | 25  | 27  | ----- | ----- | ----- |

From Table II it will be noted that the removal of nickel from the alloy sample 1 has substantially lowered the hydrogen pick-up (compare with Table I). Sample 2 indicates the increased hydrogen pick-up which results from increasing the iron content. Samples 3, 4 and 5 show the stabilizing effect, insofar as hydrogen pick-up is concerned, of increased oxygen upon alloys containing increasing amounts of iron. The corrosion resistance of the samples of the alloys shown in Table II is not affected to any substantial degree by the increased amounts of iron and oxygen therein.

The relatively high oxygen level of the alloys of this invention permits a greater tolerance in minor variations of alloying constituents, such as iron, while maintaining excellent corrosion resistance and low hydrogen pick-up. It will be understood that the above description is only exemplary and not in limitation of the invention.

We claim as our invention:

1. A workable zirconium-base alloy having a lowered

35 tive capacity for hydrogen when exposed to high temperature water or steam and containing a relatively large amount of iron therein, consisting of, from 1.3% to 1.6% by weight of tin, from 0.07% to 0.12% by weight of chromium, from 0.12% to 0.40% by weight of iron, at least 0.16%, but not exceeding 0.25%, by weight of oxygen, carbon not exceeding 0.05%, less than 0.007% nickel, the balance being zirconium and less than 0.5% by weight of incidental impurities.

#### References Cited in the file of this patent

#### UNITED STATES PATENTS

2,772,964 Thomas et al. ----- Dec. 4, 1956  
3,005,706 Thomas et al. ----- Oct. 24, 1961

#### OTHER REFERENCES

50 1. Journal of the Electrochemical Society, vol. 106, No. 3, March 1959 (pages 181-184).